

## UNITED STATES PATENT OFFICE

2,212,496

## ALLOY STEEL

Ralph P. De Vries, Menands, N. Y., assignor to  
Allegheny Ludlum Steel Corporation, Pittsburgh, Pa., a corporation of Pennsylvania

No Drawing. Original application January 10, 1939, Serial No. 250,187. Divided and this application May 27, 1939, Serial No. 276,164

3 Claims. (Cl. 75—128)

My invention relates to alloy steels which substantially maintain their hardness when repeatedly heated to temperatures of the order of 1200° to 1600° F., and air cooled. It also relates to steels which are characterized by high hardness and high strength at elevated temperatures.

One of the objects of my invention is to provide an alloy steel which, while adapted for general use, is particularly suited for those applications where resistance to scaling combined with high strength and hardness at elevated temperatures are required characteristics, and where such strength and hardness are not substantially affected by repeated heating and cooling. Such 15 steels are especially adapted for use in poppet

and sulphur may be present in the usual small quantities, and the content thereof may even be raised to as high as about 0.15%, in which case the phosphorus increases the hardness obtainable. Where phosphorus is present in more than the usual maximum of about 0.04%, small quantities of selenium, up to about 0.20%, may be added to improve the machineability of the alloy.

Below, I have set forth two specimens of my 10 alloy steels together with their hardness in the as forged condition, their hardness when air cooled from temperatures of the order of 1200° F. to 1600° F., and their hardness after reheating and air cooling from temperatures of this order. 15

| Melt No. | Analysis |     |       |      |     | As forged | Cone rockwell hardness |          |          |                                       |          |          |  |
|----------|----------|-----|-------|------|-----|-----------|------------------------|----------|----------|---------------------------------------|----------|----------|--|
|          | C        | Cr  | Mn    | N    | Co  |           | Air cooled from—       |          |          | After reheating and air cooling from— |          |          |  |
|          |          |     |       |      |     |           | 1200° F.               | 1400° F. | 1600° F. | 1200° F.                              | 1400° F. | 1600° F. |  |
| 20       | S-47     | .61 | 23.34 | 4.52 | .26 | .74       | 40/41                  | 42       | 42       | 43                                    | 40       | 40       |  |
| 25       | S-72     | .55 | 23.37 | 4.15 | .24 | .36       | 38                     | 39       | 40       | 41                                    | 34       | 35       |  |
|          |          |     |       |      |     |           |                        |          |          |                                       | 43       | 37       |  |

valves of internal combustion engines, hot work dies and similar articles which may be either forged or cast.

30 The alloying elements in my steel and the approximate percentage ranges, by weight, within which they are used to accomplish the foregoing objects are about as follows:

|    | Per cent       |
|----|----------------|
| C  | .50 to 1.25    |
| Cr | 20.00 to 26.00 |
| Mn | 2.00 to 6.00   |
| Co | .25 to 2.50    |
| N  | .10 to .50     |
| Fe | Balance        |

40 In addition to the foregoing, other elements may, of course, be incorporated in such small quantities as will not substantially impair the characteristic properties of the alloy. For example, silicon, a usual ingredient in steel, may be present up to about 0.75%, and does not in any way affect that outstanding characteristic of my alloy which is its ability substantially to maintain its hardness upon repeated heating to and air cooling from temperatures of the order of 1200° to 1600° F. The cobalt increases, in degree, the maintainable hardness, and therefore makes the steel particularly useful for hot die purposes and also for poppet valve applications. Phosphorus

It has often been found that steels which have a relatively high hardness when tested at room temperatures do not have relatively high strength or hardness when tested at elevated temperatures. The steel of my invention which has a high maintainable hardness in the temperature range of 1200° to 1600° F., has however, both high hardness and high strength at heat, the strength at a temperature of 1500° F. running consistently from 25,000 to 35,000 pounds per square inch. Such high strengths are usually found only in steels where high melting point and expensive elements such as molybdenum, tungsten or tantalum are used in fairly large proportions or where, in addition to the chromium, at least 10% to 20% of iron is replaced by nickel or manganese so that the alloy content approximates about 50% of the total composition. In my steel, however, the alloy content does not exceed from about one-fourth to one-third of the total weight of the steel.

45 My preferred quantities of chromium and manganese fall in about the middle of the ranges of these elements above specified, with carbon at least ten to fifteen points above the minimum, and nitrogen around 0.25% or more. Within these preferred ranges the alloy maintains hardness even when cooled slowly from high temperatures.

It also seems preferable when chromium is present in the extreme upper portion of its range, that both carbon and nitrogen should also be well above the minimums specified, and the manganese should be in the lower portion of its range.

This application is a division of my co-pending application Serial No. 250,187, filed January 10, 1939.

What I claim is:

- 10 1. An alloy steel characterized by the substantial maintenance of hardness upon repeated heating to temperatures of the order of 1200° to 1600° F., and air cooling; said steel containing a plurality of ingredients of which the following, in 15 the proportions stated, are the only elements necessary to attain said characteristic, carbon from 0.50% to 1.25%, chromium from 20% to 26%, manganese from 2% to 6%, nitrogen from 0.10% to 0.50%, cobalt from 0.25% to 2.5%, 20 and the balance iron.
2. An alloy steel characterized by the substantial maintenance of hardness upon repeated

heating to temperatures of the order of 1200° to 1600° F., and air cooling; said steel containing a plurality of ingredients of which the following, in the proportions stated, are the only elements necessary to attain said characteristic, carbon from 0.60% to 1.25%, chromium from 21.5% to 24.5%, manganese from 2.5% to 4.5%, nitrogen from 0.25% to 0.50%, cobalt from 0.25% to 2.5%, and the balance iron.

3. An alloy steel characterized by the substantial maintenance of hardness upon repeated heating to temperatures of the order of 1200° to 1600° F., and air cooling; said steel containing a plurality of ingredients of which the following, in the proportions stated, are the only elements 15 necessary to attain said characteristic, carbon from 0.60% to 1.25%, chromium from 24% to 26%, manganese from 2% to 4%, nitrogen from 0.25% to 0.50%, cobalt from 0.25% to 2.5%, and the balance iron.

RALPH P. DE VRIES.

20